

May 18, 1937.

H. FUNCK

2,080,965

PROCESS OF PHOTOENGRAVING

Original Filed Feb. 25, 1932

FIG. 1



FIG. 2



FIG. 3



INVENTOR.  
HARRY FUNCK.

BY  
Lockwood Lockwood Goldsmith & Galt  
ATTORNEYS.

## UNITED STATES PATENT OFFICE

2,080,965

## PROCESS OF PHOTOENGRAVING

Harry Funck, Chicago, Ill.

Application February 25, 1932, Serial No. 595,112  
Renewed October 17, 1936

16 Claims. (Cl. 95—5.6)

This invention resides in a new and novel process of producing an engraved plate for printing purposes.

The principal object of the invention is to produce such a plate through a photomechanical process which will greatly decrease the labor usually required in the known and practiced methods, decrease the time required for producing engraved plates and further, simplify the process so that the cost is minimized, while at the same time producing a plate having greater wearing qualities so as to be capable of making many more impressions.

In accordance with this invention, a halftone negative, having all possible tone-value, such as an offset negative, will produce an engraved printing plate in a very few minutes by photomechanical means, whereas it would take some time for an artist to produce a similar plate by fine or re-etching in accordance with the present practice.

The principal feature of the invention resides in applying a photo-sensitive substance having certain characteristics required for the purpose, to a plate which may be of any hard and rigid substance such as "bakelite", glass, wood, metal, fiber or the like, no particular metal or substance being required. Thus, the material from which the base or foundation of the plate is made is in itself considerably cheaper than the metals usually required for etching.

The photo-sensitive composition may be applied according to the desired depth of the engraving. For instance, for fine printing work, the screen or lines may be finer and consequently the depth of the engraving less, whereas in rough work such as news print, the screen or lines are coarse and consequently the depth of the engraving has to be greater.

The process practiced in photoengraving is carried out to the extent of producing a screen or line negative. Thereafter, this invention departs from the usual practice in that it is only necessary to apply the screen or line negative over the sensitized surface of the plate, expose the same to the light for a few minutes, and pass the plate through a developing bath and dry the same, whereupon it is ready for use. This distinguishes from the long, tedious and elaborate process usually required wherein the engraving plate has a light sensitive coating applied thereto over which the screen negative is placed, whereupon it is exposed to the light for a substantial length of time and thereupon submerged in a developing bath after which it is treated

with a protective substance to form an acid resist, which is a tedious and highly specialized art, and then submerged in the etching bath, these last two operations being repeated from one to three times, thus requiring a substantial length of time in treatment, as well as requiring most expert labor.

In addition to the reduced time and labor saving process as above pointed out, certain other material advantages in the fineness of the work and its durability result. Whereas in the practiced photoengraving process, the dots formed in the plate are to some extent undermined by the eating-in of the acid laterally, as well as downwardly, in applicant's process the substance is effected only by the light penetration, so that the tendency is for the recesses to be straight. This leaves a substantial base for the support of the dots formed in the surface as will be hereinafter more specifically pointed out. Consequently, the surface of the dots is more substantial in applicant's process than in the practiced photoengraving.

A further important advantage in respect to this feature resides in the fact that the undermining of the dots in the practiced photoengraving process tends to destroy the matrix, wax or lead molding wherein the impression thereof over the surface of the plate forces the material between the undermined dots where it spreads and tears out when removed. This difficulty is entirely eliminated in applicant's process since there is no undermining and the matrix or sheets may be readily removed without tear or mutilation.

A still further advantage resides in the fact that wherein the plate is used for direct printing, the surface of the sensitized and developed substance has a natural tendency to give off the ink to the paper more readily than the engraved metal plates used in the present practice.

Furthermore, the surface characteristics of the substance used on applicant's plate is such as to give sufficient elasticity to increase the wearing qualities as compared with the rigid inelastic surface of the copper and especially zinc surface of the photoengraved plate.

A further advantage of applicant's process is the fact that the engraving plate which may be made of various materials as above mentioned may be readily glued or cemented to the block so that it is unnecessary to tack it in position as is the usual practice with copper or zinc plates. While it may be possible to secure the copper or zinc plates in the same manner, it is difficult and

impractical to do so. Furthermore, by thus securing the plate to the block, the formation of a bevel customarily employed for tacking is eliminated.

- 5 One feature of applicant's process resides in forming the photo-sensitive substance with varying degrees of sensitivity, wherein the sensitivity of the substance will increase from the exposed surface to the base. This is for the purpose of  
10 permitting the light rays which decrease in strength as they penetrate the depth of the substance, to equally affect the substance throughout its entire depth. By providing the substance with greater sensitivity as its depth increases,  
15 the decrease in the efficiency of the light rays will be compensated for or equalized. Thus, with a short exposure, a clean-cut dot or line formation is obtained, but more important, the supporting base of the dots is strengthened. Otherwise, the  
20 strengthening effect of the light rays would not sufficiently penetrate throughout the depth of the dot to harden and thereby strengthen the base of the dot.

Another feature of the invention resides in the development of the substance after exposure in such manner as to maintain its true configuration and prevent swelling. The characteristics of the substance are such that the tendency in the development after exposure is to swell and  
30 in the subsequent drying disfigure the true formation of the dots, which objection is avoided, as will be hereinafter more fully set forth.

A further feature of the invention resides in the employment of an aniline dye in the make-up of the substance which will correct the photo-activity of the substance to prevent halation, or the spreading of the light beyond its proper boundary with the help of the usual darkened base surface, all of which will be hereinafter more specifically referred to in the following description.

Other features of the invention consist in the composition of the sensitized substance and the solution in which it is developed after exposure,  
45 as will be hereinafter pointed out, coupled with the method of applying or forming the substance on the supporting plate.

The full nature of the invention will be more clearly understood from the accompanying drawing and the following description and claims:

Fig. 1 is a perspective view of the engraving plate and block showing the finished engraved surface thereon. Fig. 2 is an enlarged section illustrative of the dots and cuts in the engraved substance. Fig. 3 is a diagrammatical illustration greatly exaggerated showing the screen negative mounted over the engraving substance.

In the drawing there is shown a substantially enlarged and exaggerated view of a printer's block 10 on which is secured an engraving plate 11 which may be cemented or otherwise secured upon the block without the usual provision of bevels or flanges to permit tacking. A photo-sensitive substance 12 is applied over the surface of the plate 11 to the thickness desired for obtaining the proper depth of engraving, depending upon the screen to be used, i. e., a fine screen or a coarse screen. The engraving plate which  
70 is preferably made of "bakelite" or any other similar material having a smooth hard surface and which may include metal, wood or the like, is usually of sixteen gauge or .0625 inch on an average in thickness, whereas the photo-sensitive  
75 engraving substance 12 for commercial purposes

is made in three thicknesses, ranging from .0015 to .008 inch in thickness.

The plate 11 with the engraving substance thereon, for commercial purposes, is manufactured in strips of convenient size and shipped to the engravers or users thereof in sealed containers so as not to be exposed to the light and may thereupon be cut to the desired dimensions for use as occasion warrants.

Wherein such plates are formed of metal, the surface thereof must be neutralized by a coating of lacquer or varnish to prevent oxidizing which, of course, is not required with non-metallic plates. Furthermore, wherein the plates are made out of metal, they cannot be readily secured by adhesion and it is, therefore, advisable to provide the usual bevel and tack them to the block. Consequently, a "bakelite" or fiber plate is recommended as being the most satisfactory.

In practising the process of engraving, the protective covering of the strip is removed in a dark room, the strip cut to the desired dimensions of the printing plate, whereupon the usual screen or line negative 13 is applied over the sensitized surface and clamped thereto in the usual vacuum frame commonly employed in the engraving industry. Thereupon, the combined negative and plate are exposed to the light in the usual manner for approximately two or three minutes, depending upon the power of the light. It is then taken to the dark room, the screen negative removed and the sensitized surface and plate submerged into a developing bath as will be hereinafter more specifically described. It is submerged in the developing bath approximately one and one-half minutes and is then dried. Immediately upon being dried, it is ready for printing.

As will be noted in Fig. 3, the dots indicated by the numeral 14 are formed in the engraving substance by recesses 15 extending throughout the entire thickness of the substance. The dots and recesses are formed by the exposure of the sensitized substance to light through the screen negative. The effect of the light thereon is to harden the substance penetrated so as to make it impervious to the developing bath.

Thus, where there is an open or white space in the screen or line negative, there will be a dot or line 14 and where there is a closed or black space, there will be formed the recess 15. That portion of the surface of the substance which is exposed to the light becomes hardened equally throughout its entire thickness and will not be affected by the solution in which the substance is developed, whereas the solution dissolves the non-exposed portion of the substance, leaving the recesses 15. In this connection, it may be noted that the light hardens and renders impervious to the solution not only the surface of the substance which it strikes, but penetrates through the entire thickness of the substance so that no dissolving thereof will occur. For this reason, the light rays striking the substance in a substantially vertical direction to its surface, the dots will be formed with substantially vertical and parallel side surfaces, presenting a clean-cut dot formation and a firm and solid base for the support thereof as distinguished from the rougher dot formation and under-cutting of the acid in the practised photoengraving process. Inasmuch as the substance 12 adheres firmly to the plate 11 and becomes for all practical purposes an integral part thereof, the dots will stand up longer under the strain thereon from many impressions and the surface, being

chemically hardened by the light, will wear indefinitely.

While it is possible that other substances may be employed for producing the sensitized engraving surface 12, the following formula is suggested as the most satisfactory now known.

With a body of chromated colloid prepared to the desired sensitivity, and preferably chromated gelatin, there is mixed a small amount of copper chloride, tartrazine dye and a lesser amount of glycerin. The chromated colloid provides the body of the sensitized substance, whereas the tartrazine dye is employed for the purpose of preventing halation, while the purpose of the glycerin is to eliminate tension of the substance. To approximately 1000 parts of the chromated colloid or gelatin, there is mixed approximately 5 parts of copper chloride, 2½ parts of tartrazine dye and 1 part glycerin. The above are thoroughly mixed 15 at about 50° C. At that temperature or thereabouts, the mixture is applied to the base plate after it has been thoroughly cleansed to remove any grease or oily film, and allowed to cool to normal temperature, whereupon it changes from a 20 liquid state to a substantially solid state and is ready for use.

The substance in liquid form at about 50° C. to 60° C. can most conveniently be applied by the usual spray gun, wherein it is sprayed over the 25 surface of the base plate to the desired thickness.

As to thickness in commercial use, it is best practice to employ three commercial thicknesses as above set forth which may be gauged by the amount of substance sprayed over a given area 30 of the surface. It is important, however, that the light ray penetrates the entire thickness of the substance with substantially the same effect on its sensitivity. One method of building up the substance so as to increase its sensitivity from the 35 exposed surface inwardly, is to provide two or more layers of substance having varying degrees of sensitivity. To accomplish this, the first or base coating of the material contains a higher percentage of a chrome salt in the colloid, whereas the 40 succeeding layers or applications of the substance have a lesser percentage of chrome. This may be accomplished by making up several solutions of the substance embodying varying percentages of chrome and using separate air guns for each solution, applying the more sensitive solution first 45 with an air gun and thereafter immediately applying the subsequent layers of substance having less or lower sensitivity, before the preceding substance has become hardened. Thus, the several 50 layers of substance are all applied in a liquid state and, therefore, become fused into one integral composition which is less sensitive toward the exposed surface.

Upon the sensitized substance becoming substantially hardened, it is then ready for packaging and commercial use as above set forth. However, to prolong its life, for shipment, storage and commercial use, a small percentage of citric acid may be employed, the acid being mixed with the ingredients of the above substance in the amount of approximately 2½ parts of citric acid to 1000 parts of colloid.

After the substance is exposed to the light, it is then developed in a subdued light, the developing solution containing ingredients such as alcohol, formalin or chrome alum, which prevent swelling of the colloid and provide a clean-cut engraved dot or line formation. A most satisfactory developer consists of any kind of alcohol (denatured) diluted to about 40%, and used at a

temperature of between 35° C. and 45° C. In effecting the development, the exposed sensitized substance on its supporting plate is immersed in the solution between one and two minutes, whereupon the unexposed surface and corresponding depth of the substance is dissolved, leaving the exposed light hardened surface and corresponding depth of the substance. After development, the substance may be further hardened if desired, by immersing in a solution of about 95% alcohol and 5% formaldehyde.

Where atmospheric or climatic conditions may react unfavorably upon the sensitized substance, it may be desirable from the commercial standpoint to adopt the following practice. This may occur in shipping the plates to tropical countries or storing the plates over a substantial length of time. In such instances, the colloid may be used without chrome salt, wherefore the substance would have no sensitivity and therefore, it would not be affected by climatic or atmospheric conditions. When ready for use, sensitivity may be imparted to the substance by immersing it in a 2½% bichromate solution containing a small amount of alcohol at 18° C. Such solution would 15 impart the necessary sensitivity to the substance, giving it the same reactive effect to light as above set forth.

In order that there may be a variation in the sensitivity of the substance through its depth 30 for the reasons and in the manner above mentioned, the substance or colloid when originally prepared and applied to the supporting plate, may contain varying amounts of a copper salt, the copper salt having the effect of increasing the 35 sensitivity when sensitized by the chrome salt solution. Therefore, in the varying depths of the colloid coating, variation in sensitivity is effected in accordance therewith.

The invention claimed is:

1. The process of making a light sensitive printing plate adapted to be processed for relief etching, consisting in applying a substantially liquid coating of light sensitive substance on the surface of a supporting base and fusing 45 therewith while still in a substantially liquid state a second substantially liquid coating of light sensitive substance of lesser sensitivity thereover.

2. The process of making a light sensitive printing plate adapted to be processed for relief etching, consisting in applying a substantially liquid coating of light sensitive substance on the surface of a supporting base, said substance including a chrome colloid for rendering the same sensitive to light, and thereafter applying a second substantially liquid coating of chrome colloid over the first coating having a lesser amount of chrome salt therein to decrease the sensitivity of the superposed coating, said second coating being applied while the first coating is still 50 in its fluid state to cause a fusing of the two 55 coatings.

3. The process of making a light sensitive printing plate adapted to be processed for relief etching, consisting in applying a coating of light 65 sensitive substance including a copper salt therein to a supporting surface, and thereupon applying a second coating having a lesser amount of copper salt, said second coating being applied over the first coating while in a plastic state.

4. The process of making a light sensitive plate adapted to be processed for relief etching, consisting in applying a coating of colloid including a copper salt therein to a supporting surface, fusing therewith while in a plastic state a sec- 70 75

ond coating of colloid having a lesser amount of copper salt, and thereafter treating the same to a bichromate solution.

5. The process of making an engraved plate 5 consisting in applying a coating of colloid over the surface of a supporting base, rendering said colloid coating sensitive to light, exposing the same to light through a negative and thereafter developing the coating in a solution of diluted 10 alcohol, and thereafter further hardening the developed coating in an alcohol formaldehyde solution, for preventing the swelling of the colloid.

6. The process of making an engraved plate 15 consisting in applying to a supporting surface a coating of light sensitive substance including a body of chromated colloid with which is mixed a relatively small amount of copper chloride, tartrazine dye and glycerin, exposing said substance to light through a negative and thereafter immersing the same in diluted alcohol as a developer.

7. The process of making an engraved plate 25 consisting in applying to a supporting surface a coating of light sensitive substance including a body of chromated colloid with which is mixed a relatively small amount of copper chloride, tartrazine dye and glycerin, exposing said substance to light through a negative and thereafter 30 immersing the same in diluted alcohol as a developer, and finally immersing the developed plate in an alcoholic formaldehyde solution for hardening the surface thereof.

8. A light sensitive substance adapted to be 35 applied to a supporting surface, including a body of chromated colloid, copper chloride, tartrazine dye and glycerin.

9. A light sensitive substance adapted to be 40 applied to a supporting surface, including one thousand parts of chromated colloid or gelatin, with which is incorporated approximately five parts of copper chloride, approximately two and one-half parts of tartrazine dye and approximately one part of glycerin.

45 10. A light sensitive substance adapted to be applied to a supporting surface, including a plurality of coatings applied one upon the other while in a plastic state, each of said coatings including chromated colloid or gelatin in which 50 is embodied a copper chloride, a tartrazine dye and glycerin, the inner coating having a greater amount of copper chloride and/or bichromate salt than the outer coating, whereby said inner coating will have greater sensitivity than the outer coating.

55 11. The process of producing an engraved plate consisting in mixing a solution of chromated colloid or gelatin of one thousand parts with approximately five parts of copper chloride, approximately two and one-half parts tartrazine dye and approximately one part of glycerin, heating the same to approximately 50° C. and applying it upon the cleansed smooth surface of a supporting base, applying thereover a sec-

ond coating having a lesser amount of copper chloride and/or bichromate salt to render the same less sensitive and while the first coating is still in a plastic state, cooling the same to a hardened state, exposing the substance to light through a negative, and thereafter immersing the same in a solution of about 40% alcohol at a temperature of about 40° C.

5 12. A process of making an engraved plate consisting in applying a coating of colloid over the surface of a supporting base, rendering said colloid coating sensitive to light, exposing the same to light through a negative, developing the coating in a solution of dilute alcohol, and thereafter immersing the developed coating in 15 a solution of alcoholic formaldehyde to further harden the surface thereof.

13. A process of making a half-tone printing plate, including applying a coating of colloid over the surface of a supporting base, said coating including copper salts, the lower portion of the coating including a greater concentration of copper salts than the upper portion of the coating, thereafter submerging the coating in a bichromate solution to render the same sensitive 20 to light, the lower portions of the coating thus being rendered more sensitive to light than the upper portions of the coating.

25 14. A process of making a half-tone printing plate, including applying a coating of colloid over the surface of a supporting base, said coating including copper salts, the lower portion of the coating including a greater concentration of copper salts than the upper portion of the coating, thereafter submerging the coating in a bichromate 30 solution to render the same sensitive to light, the lower portions of the coating thus being rendered more sensitive to light than the upper portions of the coating, exposing the same from the emulsion side to light through a 35 screened negative, and then submerging the same in a developing bath to remove the non-exposed portion of the colloid, thereby leaving half-tone dots of the exposed portion of the colloid suitable for half-tone printing.

40 15. A half-tone printing plate, comprising a rigid supporting base and half-tone dots of a developed light sensitive gelatin containing colloid on said base and possessing substantially perpendicular and clean-cut sides so that dots 45 are directly usable in half-tone printing.

16. A half-tone printing plate, comprising a rigid supporting base and half-tone printing dots resulting from subjecting a light-sensitive gelatin containing coating of a colloid on said base to exposure to light through a screened negative and the removal of the non-exposed portions of the colloid in a developing bath, the light sensitive colloid being more sensitive to light in its lower portions so as to leave the half-tone dots with substantially perpendicular straight sides 55 so as to possess sufficient rigidity to be employed directly in half-tone printing.

HARRY FUNCK.